

[54] CONTROL OF DYE MIGRATION BY  
TREATING TEXTILE WITH AQUEOUS DYE  
BATH CONTAINING AN AMIDE  
DERIVATIVE OF POLYVINYL METHYL  
ETHER/MALEIC ANHYDRIDE

[75] Inventor: **Richard F. Chambers**, Pompton  
Lakes, N.J.

[73] Assignee: **GAF Corporation**, New York, N.Y.

[22] Filed: **Dec. 3, 1973**

[21] Appl. No.: **421,130**

[52] U.S. Cl..... **8/62; 8/176;**  
260/29.2 UA

[51] Int. Cl.<sup>2</sup> ..... **D06P 1/52**

[58] Field of Search..... **8/62, 176; 260/29.2 UA**

[56] **References Cited**

UNITED STATES PATENTS

|           |        |                     |             |
|-----------|--------|---------------------|-------------|
| 2,589,951 | 3/1952 | Meier.....          | <b>8/62</b> |
| 2,800,417 | 7/1957 | Kleiner et al. .... | 260/29.2 UA |
| 3,178,385 | 4/1965 | Dinges et al. ....  | <b>8/62</b> |

*Primary Examiner*—M. J. Welsh  
*Attorney, Agent, or Firm*—Walter C. Kehm; Joshua J. Ward

[57] **ABSTRACT**

In the Thermosol and like processes in which a dye-impregnated textile material is dried prior to fixation, uncontrolled migration of the dye to the surface of the material during the drying operation is obviated by the incorporation of an antimigration additive in the aqueous dye bath liquid, said additive being an amide derivative of poly(vinyl methyl ether/maleic anhydride), said anhydride-containing copolymer having a specific viscosity of about 0.75 to about 4.5, preferably about 1.0 to about 3.5, more preferably about 2.0 to about 3.5, measured at a concentration of 1 gram per 100 ml. of methylethyl ketone at 25°C. The additive, employed within the general range of from about 0.05% to about 0.50% by weight based on the total weight of the dye bath, serves to enhance the uniformity of the dyeing operation and the color properties of the dyed textile material.

**9 Claims, No Drawings**

**CONTROL OF DYE MIGRATION BY TREATING  
TEXTILE WITH AQUEOUS DYE BATH  
CONTAINING AN AMIDE DERIVATIVE OF  
POLYVINYL METHYL ETHER/MALEIC  
ANHYDRIDE**

**BACKGROUND OF THE INVENTION**

**1. Field of the Invention**

This invention relates to the dyeing of textile materials. More particularly, it relates to a dye bath composition and to a dyeing process in which uncontrolled migration of the dye to the material surface during drying prior to fixation is minimized.

**2. Description of the Prior Art**

In commercial dyeing operations in which a textile material is impregnated with a dye by padding with an aqueous dye bath liquid, as in the conventional Thermosol process, the dye-impregnated material is commonly dried, e.g., by heating, prior to fixation of the dye. It is well known that the dye particles tend to migrate to the surface of the material during the drying operation and that such migration tends to be of an uncontrolled and random nature. Such uncontrolled migration, however, leads to an uneven dyeing, detracting from the appearance and value of the dyed textile material. As a result, various additives, including natural gums, sodium alginate and a variety of synthetic antimigrants have been proposed in order to reduce such uncontrolled migration. Many of the materials proposed in the literature were described also with respect to thickening characteristics, the terms "thickeners" and "antimigrants" commonly being employed synonymously. While many materials thus proposed as antimigrants also tend to find application in other systems as thickeners, the more persuasive teachings available suggest that the viscosity of the dye bath per se does not have any significant effect with respect to the uncontrolled dye migration problem discussed above.

While various materials have thus been proposed for antimigration additives, no such materials have found widespread acceptance because of the relatively high incremental costs associated with the use of such antimigrants, undesirable side effects that often occur as a result of the presence of particular antimigrants in specific aqueous dye bath liquor systems or a combination of these or like factors disadvantageous in the overall dyeing operation. There exists in the art, therefore, a need and a desire for less expensive, more technically efficient antimigrants having an enhanced compatibility with aqueous dye bath liquid systems for the dyeing of textile materials.

It is an object of the present invention, therefore, to provide an improved aqueous dye bath liquid capable of minimizing undesired dye migration.

It is another object of the invention to provide an improved dyeing process in which migration of the dye during drying prior to fixation is minimized.

It is a further object of the invention to provide an improved dye bath liquid having a desirable combination of effective dye migration prevention and minimal incremental cost.

With these and other objects in mind, the invention is hereinlater disclosed in detail, the novel features thereof being particularly pointed out in the appended claims.

**SUMMARY OF THE INVENTION**

Dyed textile material of enhanced quality and appearance is conveniently obtained by minimizing uncontrolled dye migration to the surface of the material during drying prior to dye fixation by the incorporation of an amide derivative of poly(vinyl methyl ether/maleic anhydride) in the aqueous dye bath liquid. The amide derivative is incorporated in the aqueous dye bath liquid in small amounts within the general range of from about 0.05% to about 0.50% by weight, based on the total weight of said dye bath. By padding an aqueous dye bath liquid containing the indicated antimigration agent therein onto the textile material being treated, it is thereafter possible to dry the dye-impregnated material to fixation without appreciable uncontrolled dye migration during the drying operation, thus preserving a greater uniformity of dyeing and permitting the production of the enhanced quality of product referred to above.

**DETAILED DESCRIPTION OF THE INVENTION**

The present invention applies to dyeing operations of the type represented by the conventional Thermosol process in which a dye is padded onto the fiber, achieving penetration into the textile fiber itself, followed by a drying of the dye-impregnated textile material and a subsequent curing or fixation of the dye as by a heat treatment operation. While numerous proposals have been made for controlling the well known migration of the dye particles to the surface of the material during the drying step, the present invention is particularly advantageous in that the improved antimigration result achieved by carrying out the dyeing operation by the use of the novel dye bath liquid herein disclosed and claimed is of an economical nature and may readily be applied to a wide variety of dyeing operations, involving a variety of different textile materials and types of dyes. This combination of effective antimigration effect, economy and flexibility of application represents a significant advance in the efforts in the art to overcome the adverse effects resulting from uncontrolled migration of dyes during essential portions of the overall dyeing operations as conveniently carried out in commercial textile dyeing applications.

The novel dye bath liquid and the dyeing process that represent differing aspects of the present invention can readily be applied in the dyeing of the various textile materials commonly dyed by the conventional Thermosol process approach. Such materials include cotton fibers, polyester fibers, polyester-cotton blends, and the like, that are thus dyed in very large quantities in commercial operations. The invention is not limited to such fibers, however, but may also be readily applied to acrylic fibers, wool and the like. It might be noted, in this regard, that the Thermosol process is commonly employed for such dyeing purposes since it is readily adapted for continuous processing involving padding, drying and curing by heat treatment or chemical means. Operations in which the material being treated is cooked or otherwise treated in the dye bath for dye fixation purposes prior to drying, on the other hand, are more commonly of a batch type operation.

One of the advantageous features of the present invention is its general application with respect to a variety of dyes, as opposed to an antimigrant approach that may only apply with respect to a particular type of dye

or a specific dye product. Thus, the present invention may be practiced in dyeing operations involving such dyes as direct dyes, vat dyes, reactive dyes, disperse dyes, acid dyes and other such dyes that are of utility, from a practical viewpoint, for textile dyeing purposes. It will be appreciated that a vast number of dyes of the various, commercially useful types are available in the art, such dyes being well known in the art, described in numerous patents and further designated by a systematic Color Index number arrangement as is well known in the art. As the invention is not limited to any specific type of dye or to any particular dye, no further descriptive matter is deemed necessary with respect to the dyes per se, apart from the general references to such dyes herein with respect to the improvements in the aqueous dye bath liquid and the dyeing process employing said novel dye bath liquid.

It will be appreciated by those skilled in the art that a variety of additives may be present in the aqueous dye bath liquid apart from the dye itself and the water with which it is associated in the dye bath liquid. Such additives include dye assistants, carriers, promoters, and the like and may be employed in conventional amounts for their usual purposes in the practice of the present invention. The dye itself may be incorporated in the dye bath liquid in amounts generally up to about 5% or more by weight based on the total weight of the dye bath. For heavier or darker shades, the dye may be employed in amounts typically of from about 2% to about 5% by weight, most typically about 3-4% by weight, whereas light shades may be achieved by employing dye concentrations of about 1/2% by weight, or less. Dye concentrations outside such ranges can also be employed within the scope of the invention, however, it also being understood that the amount of said dye bath liquid with which the textile material is impregnated, by padding, spraying, coating, printing or other means, commonly at 25-100% wet pickup, will depend upon the color requirements of any given application.

In the conventional drying operation following the impregnating of the textile material with the desired dye, the treated material is heated to any temperature and for any time sufficient to dry off the dye bath liquor, conveniently at a temperature of about 100°C. for convenience of rapid action, by any suitable means, such as by hot air, infra-red radiation, microwave oven or the like. Thus, pressures may range from below to above atmospheric, and temperatures below room temperature to over 100°C. It is during this conventional drying operation that dye migration to the material surface is known to occur, said migration tending to be uncontrolled, random and uneven, thus resulting in an uneven overall dyeing action, stripiness and a generally inferior quality of the finished product.

The antimigration additive incorporated in the aqueous dye bath liquid in the practice of the present invention serves to effectively and efficiently minimize uncontrolled dye migration during the drying operation prior to fixation. The subject additive, heretofore known and available in the art for other purposes, is the amide derivative of poly(vinyl methyl ether/maleic anhydride) believed to have the structural formula:



in which  $\text{R}_1$  and  $\text{R}_2$  are each taken from the group consisting of  $\text{H}$ ,  $\text{CH}_3$ ,  $\text{CH}_2\text{CH}_3$ ,  $\text{CH}(\text{CH}_3)_2$  and  $\text{CH}_2\text{CH}_2\text{CH}_3$  with the exception that  $\text{R}_1$  and  $\text{R}_2$  together may be a divalent unit taken from the group consisting of  $-(\text{CH}_2)_{4-6}$  and  $(-\text{CH}_2\text{CH}_2)_2\text{O}$ . The parent anhydride-containing copolymer has a specific viscosity of from about 0.75 to about 4.5 preferably about 1.0 to 4.0, more preferably about 2.0 to 4.0, measured at a concentration of about 1 gram per 100 ml. of methyl-ethyl ketone at 25°C. Illustrative of the amines that can be used in making the subject amide derivatives are ethyl amine and diethyl amine.

The subject antimigration additive will generally be incorporated in the aqueous dye bath liquid in an amount within the range of from about 0.05% to about 0.50% by weight, based on the total weight of the dye bath liquid, with the additive concentration being commonly in the range of from about 0.10% to about 0.25% by weight. As indicated above, said additives are generally known in the art and available from GAF Corporation, the additives not having been previously employed or considered with respect to the dye migration problem discussed herein. With regard to the additive materials per se, their preparation and prior applications, reference is herein made to U.S. Pat. Nos. 1,976,679, Re. 23,514, and 2,746,837. As the additives employed in the practice of the invention and their production are known and available in the art, detailed information concerning the preparation of the additive compounds is not deemed necessary herein, the present invention being directed to the dye bath liquids and methods of dyeing herein disclosed and claimed in which such known compounds are employed for antimigration purposes.

It should be noted that the pH of the aqueous dye bath liquid of the invention can generally vary over rather broad limits, although it will be appreciated that optimum pH limits will pertain with respect to particular dye bath-textile systems. If the dye bath liquid is too basic in nature, however, the amines may tend to be driven off. For this reason, the pH of the dye bath will generally be less than about 9, e.g., in the range of from about 4 to about 9, typically from about 6 to about 8, preferably about 7, although some dye-textile applications may be operative outside the indicated limits.

After the textile material being treated has been impregnated with a desired dye by contact with the aqueous dye bath liquid of the present invention, and the material has been dried by conventional means, the dye is fixed by heat or other means as by chemical action. Such fixation techniques are well known and established in the textile dyeing art. The present invention is not limited to any such technique, but can be practiced with dye fixation by any conventional technique following the drying of the dye-impregnated fiber. Illustratively, curing may be carried out at temperatures of about 120° to 230°C for about 3 minutes to 15 seconds, depending on the fabric, the dye, and the like.

The present invention is hereinafter illustrated by reference to specific illustrative examples, it being understood that such examples are presented to provide a further understanding as to the advantages of the invention and should not be construed as limiting the scope thereof as set forth in the appended claims. It will also be understood that all parts and proportions referred to herein and in the appended claims are by weight unless otherwise so indicated.

#### EXAMPLE 1

5 g. of poly(vinyl methyl ether/maleic anhydride),

specific viscosity 3.77, was slurried in 92.6 g. of water. 2.4 g. of a 70% by weight solution of ethylamine in water was added and mixed. The temperature of the mix was increased to 90°C., at which temperature the mix cleared. The resulting amide additive solution was then cooled to room temperature and employed in a dye bath liquid having the following composition: Indanthrene olive T3R paste, GAF Vat Black 25, Color Index No. 69525, 3.0 g.; the additive solution prepared above, 4.5 gr.; Gaftex CD 169, a biodegradable anionic surfactant, wetting agent, 0.15 gr.; and water, 92.35 gr. After mixing of these ingredients, the pH of the resulting aqueous dye bath liquid was adjusted to 6.6 with a few drops of glacial acetic acid.

For purposes of illustrative dyeing tests, a 5 × 5 inches swatch of 100% cotton twill was padded with the indicated dye bath at 55% wet pickup by weight of dry material. The thus-treated material was placed flat on a glass plate and dried by means of an electric hot air gun held with the nozzle 11 inches above the dye impregnated swatch for 5 minutes. In this manner, the unevenness of drying that occurs in ordinary commercial operations was exaggerated and emphasized in order to illustrate the advantageous effect achieved in the practice of the invention. The reflectance of the two sides of the swatch was measured, after such drying and conventional fixation, with a Hunterlab Spectrometer calibrated to read 100% reflectance for an untreated swatch of cotton twill, increasing lower percentages thus indicating an increased color effect resulting from an increased dye content at the surface of the material. The reflectances thus obtained for the swatch thus dyed in accordance with the invention were 48.1% at the top of the swatch and 57.0% at the bottom, the lower reflectance at the top resulting from the tendency for dye migration to occur during drying and the predetermined positioning of the drying means on top of the swatch as indicated above.

A second swatch sample was treated identically as above except that distilled water was substituted for the additive solution. Under the same drying conditions, the reflectances obtained on top of the swatch and on the bottom thereof were 48.9% and 65.0% respectively. The considerably larger variation in top and bottom reflectance values obtained in the latter test, as compared with that carried out in accordance with the present invention, is indicative of the uneven dyeing that results from uncontrolled and uneven dye migration that inevitably occurs in ordinary commercial dyeing operations of the type herein discussed.

#### Example 2

The procedures as set forth in Example 1 were essentially followed in the preparation and use of an additive solution made from 5 grams of the indicated poly(vinyl methyl ether/maleic anhydride), 2.7 g. of diethylamine and 92.3 g. of water. Likewise, the dye bath liquid is prepared in the same manner as Example 1, except that the additive solution prepared from the ingredients listed above, including the same amount of wetting agent, was employed in place of the ingredients and proportions in said Example 1.

Upon treatment of a swatch with this dye bath liquid, drying and fixing said dye, as in Example 1 above, the reflectance values obtained were 48.0% at the top of the swatch and 58.1% at the bottom. As in Example 1, the significant reduction in the reflectance variation between the top and bottom of the treated swatch

under the predetermined uneven drying conditions employed is indicative of the control of dye migration the present invention makes possible, the minimizing of uncontrolled dye migration and the resulting enhancing of the uniformity and general quality of textile products dyed in accordance with the present invention.

In dyeing operations employing a commonly used textile gum antimigrant, i.e., Superclear 100-N, the effective antimigration action of the present invention has been found to require, on a weight to weight basis, very considerably more of the active solid antimigrant content as that required in the practice of the present invention. Coupled with a considerably lower unit cost for the antimigrant of the present invention, the use of the aqueous dye bath liquid of the present invention permits the production of improved textile products, having enhanced uniformity of color, at a very significantly reduced cost as compared with that required when conventional textile gums are employed for antimigration purposes. The present invention satisfies the needs and requirements of the dyeing art, therefore, in a manner highly advantageous from an overall technical and economic viewpoint.

As indicated above, commercially applicable techniques for the drying of dye-impregnated textile materials are always subject to variations and degrees of unevenness that tend to result in uncontrolled, random and uneven migration of the dye to the surface of the treated material. Even under highly uneven drying conditions, beyond those likely to be encountered in quality commercial applications, the present invention tends to minimize such uncontrolled and uneven dyeing migration. As a result, textile material dyed in accordance with the practice of the present invention has an enhanced evenness and quality of color, avoiding the unevenness and stripiness that obtains in inferior dyeing operations and products. As the highly desirable results obtainable by means of the present invention are accomplished in an advantageously economic manner, with desired flexibility of application, the invention herein described and claimed represents an important advance in the textile dyeing art, and the production of premium quality textile products.

I claim:

1. In an aqueous dye bath liquid suitable for the impregnating of textile material with said dye, the improvement comprising the incorporation in said dye bath of a polymeric antimigration additive in an amount within the range of from about 0.05% to about 0.50% by weight, based on the total weight of said dye bath, said additive being the amide derivative of poly (vinyl methyl ether/maleic anhydride) having the structural formula:



in which  $\text{R}_1$  and  $\text{R}_2$  are each taken from the group consisting of  $\text{H}$ ,  $\text{CH}_3$ ,  $\text{CH}_2\text{CH}_3$ ,  $\text{CH}(\text{CH}_3)_2$  and  $\text{CH}_2\text{CH}_2\text{CH}_3$  with the exception that  $\text{R}_1$  and  $\text{R}_2$  together may be a divalent unit taken from the group consisting

of  $-(\text{CH}_2)_{4-6}-$  and  $(-\text{CH}_2\text{CH}_2)_2\text{O}$ , the poly(vinyl methyl ether/maleic anhydride) having a specific viscosity of from about 0.75 to about 4.5 measured at a concentration of about 1 gram per 100 ml of methyl-ethyl ketone at 25°C, the presence of said additive serving to minimize uncontrolled dye migration to the surface of the dye-impregnated textile material during the drying of said material prior to fixing, thus enhancing the uniformity of the dyeing operation and the color properties of the dyed textile material.

2. The aqueous dye bath of claim 1 in which said additive is present in an amount within the range of from about 0.10% to about 0.25% by weight based on the total weight of said dye bath.

3. The aqueous dye bath liquid of claim 1 in which  $\text{R}_1$  is H and  $\text{R}_2$  is  $\text{CH}_2-\text{CH}_3$ .

4. The aqueous dye bath liquid of claim 1 in which  $\text{R}_1$  and  $\text{R}_2$  are both  $\text{CH}_2-\text{CH}_3$ .

5. A process for the dyeing of textile materials essentially without uncontrolled migration of the dye to the surface of the material during the drying of the impregnated material prior to dye fixation, consisting essentially of:

a. impregnating the textile material being treated

10

15

20

25

with an aqueous dye bath liquid as defined in claim

1;

b. heating said dye-impregnated textile material to remove aqueous dye bath liquid therefrom, thus drying said material; and

c. fixing said dye in said dried, dye-impregnated textile material, whereby the antimigration additive serves to minimize uncontrolled dye migration to the surface of the textile material during the drying operation, thus enhancing the uniformity of the drying operation and the color properties of the dyed textile material.

6. The process of claim 5 in which said additive is present in an amount within the range of from about 0.10% to about 0.25% by weight based on the total weight of said dye bath.

7. The process of claim 5 in which  $\text{R}_1$  is H and  $\text{R}_2$  is  $\text{CH}_2-\text{CH}_3$ .

8. The process of claim 5 in which  $\text{R}_1$  and  $\text{R}_2$  are both  $\text{CH}_2-\text{CH}_3$ .

9. The process of claim 5 in which said textile material being treated is taken from the group consisting of cotton, polyester and cotton-polyester blend fabrics.

\* \* \* \* \*

30

35

40

45

50

55

60

65